# EUROPEAN PATENT SPECIFICATION

(11) **EP 0 408 803 B1**
(45) Date of publication and mention of the grant of the patent: **12.01.1994**
(21) Application number: 89117234.8
(22) Date of filing: 18.09.1989
(51) Int. Cl.: D21C 9/10, D21C 9/14

(54) **Procedure for the bleaching of sulphate pulp**
Verfahren zum Bleichen von Sulfatzellstoff
Procédé de blanchiment de pâte au sulfate

(30) Priority: 10.07.1989 FI 893338
(43) Date of publication of application: 23.01.1991
(73) Proprietor: ENSO-GUTZEIT OY, FIN-00160 Helsinki (FI)
(72) Inventor: Vaheri, Marja, SF-02210 Espoo (FI); Miikki, Kari, SF-55100 Imatra (FI)
(74) Representative: Weitzel, Wolfgang, Dr.-Ing.

(56) References cited:
- DE-A- 3 636 208
- TAPPI, vol. 67, no. 10, October 1984, pages 31-33; R. FARRELL: "Biocatalystshold promise of better pulp quality"

## Description

The present invention relates to a procedure for the bleaching of pulp, in which procedure an oxidating bleaching chemical containing chlorine is used.

Especially pulp obtained from a sulphate pulping process is of brown colour, which is mainly due to the lignin remaining in the pulp. Lignin is removed from the pulp by bleaching, which is generally a process consisting of several stages. During this process, the pulp is treated alternately with oxidizing, lignin-degrading chemicals and chemicals dissolving the degradation products. Oxidizing agents commonly used are chlorine-containing chemicals and oxygen, whereas alkali solutions are used for eliminating the degradation products.

In the reactions occurring in bleaching using chlorine-containing chemicals, lignin is converted into organic chlorine compounds, which remain in the spent bleach liquor. Spent bleach liquors are a problem in regard of environmental protection because of the possible toxic nature of the organic chlorine compounds contained in the liquors. Moreover, the chemical oxygen demand in spent bleach liquors reaches detrimental levels.

The spent bleach liquors causing the worst environmental pollution load are produced in the washing stages following the first chlorination and the first alkali treatment in the bleaching process. To reduce the pollution load, various methods have been employed, including the use of chlorine dioxide instead of chlorine gas, the use of oxygen as an oxidating chemical in the first bleaching stage, and biological purification of the spent bleach liquor. However, these methods have not yielded completely satisfactory results. Although the amounts of chlorophenols and other toxic-chlorine compounds in the spent bleach liquor have been significantly reduced by using chlorine dioxide and employing oxygen bleaching, it has not been possible to achieve a sufficient reduction in the chemical oxygen demand values of the effluents. Therefore, the methods referred to have required the employment of efficient biological purification.

DE-A-3 636 208 (see also WO-A-8 803 190) discloses a method based on the treatment of natural or mechanically modified pulp raw material. The process is described with one example in which straw is treated with enzymes in order to dissolve the lignin. It has to be noted that there are significant differences of the structure of straw lignin and wood lignin (Wei He Diesheng Tai and Stephen Y. Lin, 1991). In addition, the known process calls for a pretreatment, whereby straw was pretreated with 1-2 % NaOH for 24-28 hrs, and was grinded before addition of enzyme. Such pretreatment is technically difficult, and not suitable for removing of the wood lignin.

Int. Cont. Biotechnol. Pulp & PaperInd. (1986), 67-69, concerns the enzyme treatment of a cellulose mass concentrating mainly on the use of the hemicellulases. By the use of hemicellulases chemical savings in the chlorine bleaching have been obtained, but the use of oxidases and ligninases is based on completely different reaction mechanisms which are difficult to rule (Lehninger). In the publication it is mentioned that the use of peroxidases was tested with birch and pine peroxyacid pulps. The pulps produced by the peroxyacid treatment differ substantially from the conventionally produced pulps. Additionally, the enzymed tested were peroxidases or ligninasees. In the publication it is also mentioned that the lignin content of the pulp dit not change substantially as a result of the treatment. This shows how difficult it was to reduce the lignin content with enzymes.

Tappi, Vol 67, 1984, 31-33, the possibilities of "lignin-degrading enzymes" is discussed in general terms. The publication does not contain any concrete knowledge of the subject to be discussed.

The object of the present invention is to achieve a sulphate pulp bleaching procedure that enables the toxic content and chemical oxygen demand of the spent bleach liquor to be reduced so as to reduce the need for purification of the liquor. This object is achieved by the characterizing part of claim 1.

It has been observed in earlier investigations that by using enzymes degrading hemicellulose it is possible to separate lignin and/or hemicellulose from cellulose and thus make the pulp more easily bleachable in the subsequent bleaching stages. This effect has not been observed before in conjunction with the use of lignin-degrading enzymes.

According to the invention, it has now been observed that a treatment with a suitable redox enzyme reduces the amount of chlorine chemicals required for bleaching, thereby also reducing the amounts of organic chlorine compounds left in the spent bleach liquor.

According to the invention, the redox potential of the enzymatic reaction should be below 400 mV, preferably below 250 mV. Suitable redox enzymes are phenoloxidases, such as the laccase produced by the white-rot fungus.

Except for the enzyme treatment, the bleaching of pulp by the procedure of the invention can be performed in the conventional manner by employing alternate oxidation and alkali stages and washing the pulp after each of these stages to remove the bleaching chemicals and degradation products.

The enzyme treatment as taught by the invention is preferably carried out in a temperature range of 10-90 °C, the most suitable range being 40-80 °C, with pH values in the range 3.0-10.0, preferably 4.0-8.0. The enzyme used is the lignin-modifying oxidation-reduction enzyme, laccase, as mentioned above.

The invention also concerns the use of a lignin-modifying enzyme, e.g. the laccase produced by the white-rot fungus, in the bleaching of sulphate pulp using an oxidating bleaching chemical containing chlorine.

In the following, the invention is described in greater detail by the aid of examples of embodiments based on laboratory experiments.

### Example 1

A diluted enzyme mixture of laccase produced by the Trametes hirsuta white-rot fungus was added to 220 g of dry matter obtained from pine sulphate pulp (with a dry matter content of 30%) so that a mixture with a consistency of 10% and a laccase activity of 60 U/kg of pulp dry matter was obtained. The temperature in the enzyme treatment was 55 °C and the duration of treatment 2 h. After the enzyme treatment the pulp wax filtered in a Buchner funnel and the pulp cake obtained was washed with ion-exchange-treated water so that a wash ratio of 20 was obtained.

For reference, a corresponding portion of pulp was treated in the same way except that no enzyme was added.

Next, both the pulp quantity which had undergone enzyme treatment and the reference portion were bleached by a process consisting of five successive stages of oxidation and bleaching. In the first stage, the chemicals used were chlorine (90%) and chlorine dioxide (10%), in the second stage sodium hydroxide, in the third stage chlorine dioxide, in the fourth stage sodium hydroxide and in the fifth stage chlorine dioxide.

The consumption of bleaching chemicals and the analysis results representing the quality of the bleached pulp are presented in Table 1.

The experiment shows that by using a lignin-modifying enzyme, i.e. laccase, a substantial reduction in the amount of chlorine has been achieved.

## Claims

1. Procedure for the bleaching of sulphate pulp, said procedure using an oxidating bleaching chemical containing chlorine, **characterized** in that, before oxidation, the pulp is subjected to an enzyme treatment in which a lignin-modifying oxidation-reduction enzyme is used, and in that the enzyme used is a lignin-modifying phenoloxidase, such as the laccase produced by the white-rot fungus.

2. Procedure according to claim 1, **characterized** in that the redox potential of the enzymatic reaction is below 400 mV, preferably below 250 mV.

3. Procedure according to any one of the preceding claims, **characterized** in that the pulp is treated with a phenoloxidase, e.g. laccase, and washed before the first oxidation phase.

4. Procedure according to any one of the preceding claims, **characterized** in that the bleaching chemical used in the oxidation phases is chlorine dioxide or a mixture of chlorine dioxide and chlorine gas, and that between the oxidation phases the pulp is treated with an alkali.

5. Procedure according to any one of the preceding claims, **characterized** in that the enzyme treatment is carried out in a temperature range of 10-90 °C, preferably 40-80 °C, with pH values in the range 3.0-10.0, preferably 4.0-8.0.

6. Procedure according to any one of the preceding claims, **characterized** in that the procedure is used for the bleaching of softwood pulp, e.g. pine sulphate pulp.

7. Use of a lignin-modifying oxidation-reduction enzyme wherein the enzyme used is a phenoloxidase, e.g. the laccase produced by the white-rot fungus in a sulphate pulp bleaching process using an oxidating bleaching chemical containing chlorine.

## Patentansprüche

1. Verfahren zum Bleichen von Sulfatzellstoff, unter Anwendung einer oxidierenden Bleich-Chemikalie, die Chlor enthält, dadurch gekennzeichnet, daß der Zellstoff vor der Oxidation einer Enzymbehandlung unterworfen wird, bei welcher Lignin-modifizierendes Oxidations-Reduktions-Enzym verwendet wird, und daß das verwendete Enzym eine Lignin-modifizierende Phenoloxidase ist, wie Laccase, erzeugt durch den weiß-roten Fungus.

2. Verfahren nach Anspruch 1, dadurch gekennzeichnet, daß das Redox-Potential der enzymatischen Reaktion unter 400 mV liegt, vorzugsweise unter 250 mV.

3. Verfahren nach einem der vorausgegangenen Ansprüche, dadurch gekennzeichnet, daß der Zellstoff mit einer Phenoloxidase behandelt wird, z. B. Laccase, und vor der ersten Oxidationsphase ausgewaschen wird.

4. Verfahren nach einem der vorausgegangenen Ansprüche, dadurch gekennzeichnet, daß die bei den Oxidationsphasen verwendete Bleich-Chemikalie Chlordioxid oder ein Gemisch aus Chlordioxid und Chlorgas ist, und daß der Zellstoff zwischen den Oxidationsphasen mit einem Alkali behandelt wird.

5. Verfahren nach einem der vorausgegangenen Ansprüche, dadurch gekennzeichnet, daß die Enzymbehandlung in einem Temperaturbereich von 10-90° C, vorzugsweise 40-80° C, bei pH-Werten im Bereich von 3,0 - 10,0, vorzugsweise von 4,0 - 8,0 durchgeführt wird.

6. Verfahren nach einem der vorausgegangenen Ansprüche, dadurch gekennzeichnet, daß das Verfahren angewandt wird zum Bleichen Nadelholzzellstoff, z. B. von Piniensulfatzellstoff.

7. Anwendung eines Lignin-modifizierenden Oxidations-Reduktions-Enzyms, wobei das verwendete Enzym eine Phenoloxidase ist, z. B. Laccase, erzeugt durch den weiß-roten Fungus, in einem Sulfatzellstoff-Bleichprozess unter Anwendung einer oxidierenden Bleich-Chemikalie, die Chlor enthält.

## Revendications

1. Procédé de blanchiment de pâte au sulfate, utilisant un produit chimique blanchissant oxydant contenant du chlore, caractérisé en ce qu'avant l'oxydation, la pâte est soumise à un traitement enzymatique dans lequel on utilise une enzyme d'oxydoréduction modifiant la lignine, et en ce que l'enzyme utilisée est une phénoloxydase modifiant la lignine, telle que la laccase produite par le champignon de la pourriture blanche.

2. Procédé selon la revendication 1, caractérisé en ce que le potentiel redox de la réaction enzymatique est inférieur à 400 mV de préférence inférieur à 250 mV.

3. Procédé selon l'une quelconque des revendications précédentes, caractérisé en ce qu'on traite la pulpe avec une phénoloxydase, par exemple la laccase et qu'on lave avant la première étape d'oxydation.

4. Procédé selon l'une quelconque des revendications précédentes, caractérisé en ce que le produit chimique de blanchiment utilisé dans les phases d'oxydation est le dioxyde de chlore ou un mélange de dioxyde de chlore et de chlore gazeux, et qu'entre les phases d'oxydation on traite la pâte avec un alcali.

5. Procédé selon l'une quelconque des revendications précédentes, caractérisé en ce que le traitement par enzyme est réalisé dans un intervalle de température de 10-90°C, de préférence 40-80°C avec des pH compris entre 3,0-10,0, de préférence 4,0-8,0.

6. Procédé selon l'une quelconque des revendications précédentes, caractérisé en ce qu'on utilise le procédé au blanchiment de la pâte de résineux, par exemple de la pâte de pin au sulfate.

7. Utilisation d'une enzyme d'oxydoréduction modifiant la lignine où l'enzyme utilisée est une phénoloxydase, par exemple la laccase produite par le champignon de la pourriture blanche, dans un processus de blanchiment de pâte au sulfate utilisant un produit chimique blanchissant oxydant contenant du chlore.
